

Nov. 12, 1929.

D. C. CHISHOLM ET AL

1,735,420

METHOD OF TREATING SILK CONTAINING WOOL MATERIALS

Filed May 12, 1926



INVENTORS  
Douglas C. Chisholm and  
BY John A. Hannum.

Day, Oberlin & Day  
ATTORNEYS.

## UNITED STATES PATENT OFFICE

DOUGLAS C. CHISHOLM AND JOHN A. HANNUM, OF CLEVELAND, OHIO, ASSIGNORS TO  
GEORGE E. COLLINGS, TRUSTEE, OF CLEVELAND, OHIO

## METHOD OF TREATING SILK-CONTAINING WOOL MATERIALS

Application filed May 12, 1926. Serial No. 108,505.

This invention relates to the utilization of wool mixed scrap or waste material, and particularly mixed wool and silk. It has heretofore been known that if scrap containing 5 wool and cotton be treated with sulphuric acid, or with hydrochloric acid gas, the cotton fibers are destroyed and the wool is left available to be worked up for re-use. It has also 10 been known that if mixed wool and artificial silk be treated with hydrochloric acid, the artificial silk is destroyed and the wool is not. The artificial silk is a form of cellulose and chemically is allied in general with cotton. Where wool is mixed with natural silk 15 however, it has heretofore been considered as impossible to eliminate such silk without also harming the wool. In fact the wool and silk are chemically both of protein character and it has heretofore been thought impossible to 20 act upon one without likewise affecting the other. In our work on this problem, we have now found however, that silk can be destroyed and the wool be left for re-use, and our procedure makes possible the working up 25 of waste wool and silk which was heretofore a loss so far as the recovery of the wool was concerned.

To the accomplishment of the foregoing and related ends, the invention, then consists 30 of the procedure and means hereinafter fully described, and particularly pointed out in the claims, the annexed drawing and the following description setting forth in detail certain features embodying the invention, such dis- 35 closed features constituting however, but one of various ways in which the principle of the invention may be used.

In said annexed drawing:—

Fig. 1 is a semi-diagrammatic vertical sec- 40 tional view taken longitudinally through an apparatus suitable for carrying out the invention; and Fig. 2 is a section taken on the plane indicated by line II—II, Fig. 1.

In proceeding in accordance with our in- 45 vention, material containing wool and natural silk is treated with an agent which exercises a differential disintegrating action, the silk being the portion attacked. The material is subjected to the action of hydrogen 50 chloride in solution, for instance most usually

a solution in water, a solution of about 30 per cent ordinarily being suitable. While sub- 55 mersion in a vat of hydrochloric acid may in some cases be desirable, we generally prefer to feed the wool and silk material or scrap to a conveyor, as endless conveyor 1, while acid from a tank 2 is sprayed thereon. The conveyor is of rubber or other suitable acid-proof material, supported by rolls 3, 4, one or both being driven from a suitable source of power, 60 and intermediate rollers 5 may be utilized for additional support if desired. A convenient feed arrangement is a hopper 6 having a conveyor 7 for supplying material to the belt. It is desirable to enclose the conveyor 1 with a 65 housing 8 and at the lower part of the housing, drains 9, 10 and 11 may be provided, these being respectively arranged under the areas supplied by the tanks 2, 12 and the water inlet 13. Spray heads may be em- 70 ployed for these respective sources of liquid, but preferably one or more perforated pipes O is provided in the upper portion of the housing, these being perforated in a manner to allow the fluid fed from the tanks or water 75 line to spray or sprinkle down over the material as carried along by the endless conveyor. Advantageously partitions 14 and 15 may be arranged to divide the casing up into compartments A, N and W, and in this man- 80 ner the respective zones of treatment may be kept separated and as further provision, a pair of squeeze rolls 16, 17 is desirably placed at the discharge end of each compartment.

The material to be treated is put into the 85 hopper 6 from which it is fed out to the endless conveyor 1, and hydrochloric acid is sprayed upon it from the tank 2, the valves therefrom being suitably regulated to allow an adequate supply of the acid to the sprayer 90 and excess acid is drained off by the drain 9 and may be returned by the pump 18 through a pipe 19 to the tank 2. After passing through the first set of squeeze rolls 16, 17, the material is now again sprayed with a 95 neutralizing solution from the tank 12. This solution is an alkali and conveniently may be a solution of sodium hydroxide of suitable strength for convenient neutralization, for instance about 5 per cent. Surplus solution 100

here again may be picked up by the pump 20 and returned through a pipe 21 to the tank 12. After passing through the second set of squeeze rolls, the material is now washed in the compartment W, water being supplied through the control line 13 from the supply main 22, the drainage from this compartment being taken off at 23 to the sewer. The material now passes through the final set of squeeze rolls and is discharged and may be finally dried, and if desired worked through a picker and a beating device. The wool left is ready to be worked up for further use as may be desired.

25 When it is desired to rinse out the acid or the neutralizing solution respectively from the compartments A or N, the control valves 24 or 25 and the cut off valves for the tanks may be manipulated so as to allow water from 20 the main 22 to pass through the feed line to the spray tubes as desired. Instead of a plurality of control valves in connection with the tanks and the water line, it is desirable in some cases to substitute a simple three-way 25 control valve.

Other modes of applying the principle of the invention may be employed, change being made as regards the features herein disclosed, provided the steps or means stated by any 30 of the following claims or the equivalent of such stated steps or means be employed.

We therefore particularly point out and distinctly claim as our invention:

1. A process of the character described, 35 which comprises destroying the silk in a mixture of silk and wool, by treating the same at ordinary temperature with hydrogen chloride in solution.

2. A process of the character described, 40 which comprises subjecting a mixture of wool and silk to the action of a strong solution of hydrogen chloride in water.

3. A process of the character described, 45 which comprises destroying the silk in a mixture of silk and wool by subjecting such mixture to the action of strong hydrochloric acid at ordinary temperature, and eliminating surplus acid.

4. A process of the character described, 50 which comprises subjecting a mixture of wool and silk to the action of hydrochloric acid at ordinary temperature, neutralizing with dilute caustic soda solution, and washing.

5. A process of the character described, 55 which comprises spraying a mixture of wool and silk with hydrochloric acid of about 30 per cent concentration, wringing the material, spraying thereon a solution of sodium hydroxide of about 5 per cent, wringing the 60 material, washing with water and drying.

Signed by us this 1st day of May, 1926.

DOUGLAS C. CHISHOLM.  
JOHN A. HANNUM.